

Sept. 12, 1944.

H. R. CLARK

2,358,056

MANUFACTURE OF PAPER FOR PHOTOGRAPHIC PURPOSES

Filed July 27, 1940



HALFORD R. CLARK

INVENTOR

*H. M. Perrins*  
BY *Daniel J. Mayne*  
ATTORNEYS

## UNITED STATES PATENT OFFICE

2,358,056

MANUFACTURE OF PAPER FOR  
PHOTOGRAPHIC PURPOSES

Halford Rogers Clark, Rochester, N. Y., assignor  
to Eastman Kodak Company, Rochester, N. Y.,  
a corporation of New Jersey

Application July 27, 1940, Serial No. 348,013

5 Claims. (Cl. 95—8)

This invention relates to the manufacture of paper for photographic purposes in which barium sulfate, dispersed in polyvinyl alcohol, is employed as the baryta coating.

In order to make ordinary paper suitable for use in the photographic industry, it must ordinarily be coated with a suspension of sulfate of barium or blanc fixe in an aqueous solution of a binding material, such as gelatin. This coating serves a double purpose. On one hand it prevents the infiltration of a photographic emulsion thereon into the fiber of the paper, on the other hand, it protects the photographic emulsion against the action of impurities contained in the paper. In the case of photographic emulsions in which other substances than gelatin are employed as the carrier for the silver halide, baryta coatings consisting of blanc fixe in gelatin have been unsatisfactory due, in many cases, to the sensitizing dyes in such emulsions being drawn down, or bleeding, into the baryta coating.

One object of my invention is to provide a method of coating paper for photographic purposes with which non-gelatin silver halide photographic emulsions may be used without any bleeding of the sensitizing dye into the coating or the paper. Other objects of my invention will appear herein.

I have found that blanc fixe, dispersed in a water solution of polyvinyl alcohol containing a plasticizer, is eminently suited for coating paper to prepare it for applying a photographic emulsion thereto. I have found that by so coating paper, non-gelatin photographic emulsions, such as described in Salo Patent No. 2,110,491, Fordyce application Serial No. 221,584, filed July 27, 1938, Lowe application Serial No. 318,560, filed February 12, 1940, and U. S. Patent No. 2,286,215, will satisfactorily adhere thereto and the sensitizing dyes in those emulsions will not bleed into the baryta coating or the paper. I have found that a baryta coating of barium sulfate, dispersed in polyvinyl alcohol, on paper prevents the infiltration of a photographic emulsion thereon into the fiber of the paper and also protects the emulsion against any impurities which might be present in the paper.

The dispersion is prepared by incorporating barium sulfate or blanc fixe into a water solution of polyvinyl alcohol containing plasticizer and this dispersion is spread upon the paper in a thin coating such as by means of a spreading machine. Obviously, other methods of application may be employed if desired, such as by spraying, etc. The viscosity of the coating mate-

rial can be controlled by the viscosity of the polyvinyl alcohol which is employed and also by the ratio of blanc fixe to polyvinyl alcohol therein. The polyvinyl alcohols, having a viscosity of 2-60 cps., are ordinarily suitable for this purpose. The percentage of solids to liquids in the coating solution may be that which operates most satisfactorily. For instance, in some cases, 15% would be satisfactory to one operator, in another case, 9% would be satisfactory, while in other cases, percentages between these limits, or above or below them, might be employed. With the low viscosity polyvinyl alcohols, the amount of solvent necessary is less than with the high viscosity polyvinyl alcohols and, therefore, the percentage of solids to liquids will admit of variation over quite a wide range. The percentage of barium sulfate or blanc fixe is that necessary to give a good surface to the paper. The percentages of barium sulfate may be those ordinarily employed in the case of gelatin baryta coatings. If desired, however, even greater proportions of blanc fixe may be employed with reference to the polyvinyl alcohol, particularly where high viscosity polyvinyl alcohols are employed.

Oftentimes it may be desirable to apply more than one baryta coating to the paper so as to obtain a desired thickness or weight of baryta thereon. The applications to paper of a plurality of coatings of barium sulfate dispersed in a water solution of polyvinyl alcohol is also to be understood as within the scope of my invention.

The accompanying drawing is of a photographic paper in accordance with my invention. Upon the support of paper a layer of baryta coating is deposited, essentially consisting of baryta or barium sulfate dispersed in an aqueous solution of polyvinyl alcohol. Upon evaporation of the water, a baryta-coated paper is obtained. The photographic paper is then formed by applying a silver halide photographic emulsion layer thereto in the usual manner.

The following example illustrates the preparation of a baryta coating in accordance with my invention.

10 parts of a plasticizer which will retain water such as urea, glycerine or sorbitol was incorporated in 400 parts of a 5% solution of polyvinyl alcohol. A mixture was also prepared of 359 parts of blanc fixe (43% water), 300 parts of water and 8 parts of butyl alcohol, these all being incorporated with each other. This mixture was stirred into the solution of polyvinyl alcohol and the mixture was run through a colloid mill for about three minutes or until homogeneous.

The material contained 23% solids and 2.3% polyvinyl alcohol. Paper was coated with this dispersion by means of the spreading machine and after drying, the paper was found to be satisfactory for coating with a silver halide photographic emulsion. Although a gelatin photographic emulsion can be applied to the paper coated with baryta, my invention is particularly applicable to the preparation of photographic papers in which non-gelatin photographic emulsions are coated over the baryta coating.

In the example, a small amount of butyl alcohol was incorporated to decrease the foaming which might occur in running the mixture through a colloid mill to impart homogeneity thereto. Any compatible foaming agent may be added if the amount of foaming otherwise present is objectionable. For instance octyl alcohol may be employed in this connection. I have found that the photographic papers, in accordance with my invention in which the paper is first coated with a polyvinyl alcohol-baryta coating and then with a photographic silver halide emulsion, are stable and a sharp, clear-cut image may be recorded thereon.

I claim:

1. A photographic paper essentially consisting of paper having a coating thereon essentially consisting of barium sulfate dispersed in polyvinyl alcohol, and an overcoating of a photographic emulsion essentially consisting of silver halide and a carrier therefor selected from the group consisting of gelatin and polyvinyl alcohol, the barium sulfate coating protecting the emulsion from substances having a derogatory effect thereon.

2. A photographic paper essentially consisting of paper having a coating thereon essentially

consisting of barium sulfate, polyvinyl alcohol, and a small proportion of plasticizer, and an overcoating of a photographic emulsion essentially consisting of silver halide and a carrier therefor selected from the group consisting of gelatin and polyvinyl alcohol, the barium sulfate coating protecting the emulsion from substances having a derogatory effect thereon.

3. A photographic paper essentially consisting of paper having a coating thereon essentially consisting of barium sulfate dispersed in polyvinyl alcohol, and an overcoating of a photographic emulsion in which polyvinyl alcohol is present as the protective colloid for the silver halide, the barium sulfate coating on the paper protecting the emulsion from substances having a derogatory effect thereon.

4. A photographic paper essentially consisting of paper having a coating thereon essentially consisting of barium sulfate dispersed in polyvinyl alcohol and an overcoating of a photographic emulsion essentially consisting of silver halide, a carrier therefor essentially consisting of gelatin and a polyvinyl alcohol and a sensitizing dye, the barium sulfate coating preventing the passage of discoloring materials from one outer layer to the other.

5. A photographic paper essentially consisting of paper having a coating thereon, essentially consisting of barium sulfate dispersed in polyvinyl alcohol and an overcoating of a photographic emulsion in which gelatin is present as the protective colloid for the silver halide, the barium sulfate coating protecting the emulsion from substances having a derogatory effect thereon.

HALFORD R. CLARK.